# EUROPEAN PATENT SPECIFICATION

(11) **EP 0 020 357 B1**
(45) Date of publication and mention of the grant of the patent: **18.07.1984**
(21) Application number: 79900923.8
(22) Date of filing: 15.11.1978
(51) Int. Cl.: C22C 38/02, C22C 38/04, C22C 38/12, F16H 55/06

(54) **LOWER BAINITE ALLOY STEEL ARTICLE**
ARTIKEL AUS BAINITISCHER STAHL-LEGIERUNG
ARTICLE EN ACIER BAINITIQUE

(43) Date of publication of application: 07.01.1981
(73) Proprietor: CATERPILLAR TRACTOR CO., Peoria, Illinois 61629 (US)
(72) Inventor: RICE, Stuart L., Morton, IL 61550 (US)
(74) Representative: Wagner, Karl H., Dipl.-Ing.
(86) International application number: US7800151
(87) International publication number: WO8001083

## Description

### Technical field

This invention relates generally to a low temperature bainitic alloy steel.

### Background art

Carburized and hardened alloy steel gears are widely used for vehicle power trains in order to obtain a sufficient resistance to surface pitting and high bending loads, and thereby a generally desirable service life. However, the heat treating and processing of such gears takes a long time, uses a considerable amount of energy and, accordingly, the gears are expensive. Drastic quenching of the gears is also often required, which results in considerable distortion. Moreover, even with such extensive processing, the microstructure of the gears is inhomogeneous and the gears lack sufficient case toughness at the desired high hardness levels. Likewise, nitrided alloy steel gears are relatively brittle at relatively high hardness levels, for example, above a magnitude of about 58 on the Rockwell C hardness scale (Rc58), and do not exhibit a relatively uniform metallographic structure.

The properties of some bainitic alloy steels are very desirable as a substitute for the above- mention martensitic steels. For example, in high carbon steels low temperature bainite is more ductile than martensite at the same hardness level. But most prior art bainitic alloy steels have utilized controlled amounts of potentially critical and/or expensive materials such as chromium and nickel. Exemplary of the art in this area are the following U.S. Patents Nos.: 3,418,178 to S. A. Kulin et al on December 24, 1968; 3,303,061 to J. E. Wilson on February 7, 1967; 2,128,621 to B. R. Queneau on August 30, 1938; 3,298,827 to C. F. Jatczak on January 17, 1967; 3,348,981 to S. Goda et al on October 24, 1967; 3,366,471 to M. Hill et al on January 30, 1968; 3,418,178 to S. A. Kulin et al on December 24, 1968; 3,528,088 to H. Seghezzi et al on September 8, 1970; and 3,907,614 to B. L. Bramfitt et al on September 23, 1975. A considerable portion of the available carbon is tied up by the critical alloy in the aforementioned patent references so that a relatively coarse crystallographic texture is formed that is detrimental to the toughness and hardness of the final article. Another disadvantage is that when such critical alloys are utilized, the austenite transformation temperature is generally raised, thereby requiring increased amounts of energy and adding to the processing costs.

U.S. Patent No. 1,924,099 issued to E. C. Bain et al on August 29, 1933 describes a process known as austempering. Such process involves the steps of: a) heating a steel article above an upper critical temperature to assure a change in the morphology of the article to sub--stantially 100% austenite; b) quenching the article below approximately 540°C. (1000°F.), but above the temperature of martensite formation or the so-called martensite start (Mₛ) line; and c) holding the steel article at such an intermediate temperature for a preselected period of time sufficient to convert the morphology of the article to a form other than 100% martensite. While time-temperature-transformation (TTT) diagrams are known on various prior art steels, the alloy compositions and austempering processes resorted to have suffered two general deficiencies. Firstly, the quenching step has involved cooling at a rate such that the transforming start (Tₛ) curve of the alloy has been crossed and undesirable upper transformation products such as proeutectoid ferrite/carbide, pearlite, and upper bainite formed. This is due to a major degree to the relatively critical time period of the alloy to the usual nose portion of the transformation start curve. The undesirable crossover of such nose portion results in a loss of toughness and hardness. Secondly, the heat treat holding times sufficient to obtain substantially complete transformation have been too long, for example, five hours or more. For general commercial applications, such an extended holding period is substantially impractical and represents a considerable waste of energy and time.

Still another factor of major importance is that as the body of the article to be produced increases in thickness, its cooling rate decreases. As a consequence, although thin nails or the like having an appreciable proportion of lower temperature bainite may have been made because such articles could be rapidly cooled in a practical manner, it is believed that the prior art TTT digrams of the materials of such articles would not permit the practical production of a substantially complete lower temperature bainite morphology when the section thickness is increased to about 12 mm (1/2"), for example. Thus, the composition taught by U.S. Patent No. 3,528,088 to H. Seghezzi et al on September 8, 1970 is not desirable for an article thicker than about 12 mm (1/2") because the austempered morphology of the article would vary nonuni- formly across its cross section away from substantially complete lower bainite, and the hardness would undesirably drop below a magnitude level of about 55 to 58 on the Rockwell C scale. The anchoring device of the Seghezzi patent also undesirably utilizes the potentially critical element chromium. U.S. Patent No. 3,196,052 to K. G. Hann on June 28, 1961 is representative of another alloy steel for a thin wire that has substantially the same problems.

In some instances, such as in U.S. Patent No. 2,814,580 to H. D. Hoover on November 26, 1957, processing of certain steel alloys has been accomplished at a holding temperature which is above the level of lower bainite formation. In other instances, although a lower holding temperature may have been established, austenite, pearlite, upper bainite or matensite have been undesirably present to an excessive proportion in comparison with the lower temperature bainite, for example, above an individual or collective proportion of about 10 Vol.%.

The present invention is directed to overcoming one or more of the problems as set forth above.

### Disclosure of invention

In accordance with the present invention there is provided a bainitic steel alloy article consisting of carbon in the range of 0.65 to 0.75 Wt.%, manganese in the range of 0.60 to 0.70 Wt.%, silicon in the range of 1.20 to 2.00 Wt.%, molybdenum in the range of 0.50 to 0.60 Wt.%, optionally boron in the range of 0.0003 to 0.004 Wt.%, a plurality of residual elements individually limited to less than 0.20 Wt.% and the balance iron, said article having been heat treated to achieve a predominantly homogeneous and substantially complete low temperature bainite microstructure.

Preferred features of the invention are defined in the dependent claims.

### Brief description of drawings

Figure 1 shows a diagrammatic time-temperature-transformation diagram for a bainitic alloy steel article of the present invention and including a heat treatment processing route.

Best mode for carrying out the invention The composition of the low temperature bainitic alloy steel article according to the present invention consists essentially of the following elements in the proportions indicated:

Preferably, but I believe not essentially, boron in the broad range of 0.0003 to 0.004 Wt.% is controllably added to the above-designated composition. More particularly, a boron range of 0.002 to 0.0035 Wt.% is preferred, and the most desirable amount is about 0.003 Wt.%.

In the composition of the novel alloy steel of this invention carbon (c) is present in the relatively high amounts indiciated to impart the desired strength and hardness throughout the body of the article. Carbon is an austenite former, and is present in the minimum amount stated to assure that a relatively uniform through-hardness value of a magnitude in excess of about R_{c}56 on the Rockwell C hardness scale can be obtained in the finished article. Below this minimum value the alloy would lack sufficient hardness and strength. Above the maximum stated value the alloy would become less ductile and/or too brittle, and the amount of carbon present would undesirably contribute to the formation of free carbides. Moreover, the range of carbon set forth assures that substantially complete transformation to low temperature bainite can be positively obtained.

Manganese (Mn) is also an austenite former and ferrite strengthener. Below the minimum established value the strength and hardness of the article produced would be lower than that desired, and there would not be enough manganese to tie up at least some of the sulfur usually present in residual amounts and to form manganese sulfide rather than undesirable iron sulfide. Above the maximum established value the ductility of the article would be lowered excessively.

Silicon (Si) is also a ferrite strengthener and is effective in the amounts indicated to assure the desired tensile strength and hardness of the final low temperature bainite alloy, as well as for grain size control. Below the stated minimum value there would be insufficient silicon for deoxidation purposes and for the desired level of hardness in the range of magnitude above about R_{c}56. Above the stated maximum value the toughness decreases to the point where excessive embrittlement occurs, and graphite tends to form.

Molybdenum (Mo) reduces graphitization, is a ferrite strengthener, and provides the desired hardenability characteristics to the low temperature bainite alloy. In general, the stated amounts of carbon, manganese, silicon, and molybdenum serve to lower the martensite start (Mₛ) transformation portion of the process route permitting the lower bainite transformation to occur at a relatively'low holding temperature for increased hardenability of the article and at a savings in energy. Furthermore, these four elements optimize the position of the transformation start curve so that quenching does not have to be achieved at an excessive rate. More specifically, the nose portion of the transformation start curve is thereby desirably located to the right on the TTT diagram sufficient to allow quenching of articles of thicker cross section at a more practical rate that will minimize distortion of the article and still result in relatively uniform through-hardening thereof. Below the minimum value of molybdenum hardness undesirably decreases and the transformation start curve is too far to the left so that quench rate problems arise. On the other hand, above the stated maximum value of molybdenum the transformation completed curve is located too far to the right on the TTT diagram, resulting in an extended required holding time of above two hours and a corresponding waste of energy.

Boron (B) improves bainite hardenability. The addition of boron (B) is preferred because the boron plus molybdenum plus silicon conserve these elements and provide a more advantageous rightward position of the transformation start curve and to thereby permit more practical cooling rates for articles of various thickness during austempering. Boron and molybdenum and possibly silicon retard the polygonal ferrite reaction without retarding the bainitic ferrite reaction. Furthermore, the boron acts as an intensifier from the standpoint that it intensifies the reaction of the other major elements. Boron is present in the minimum amount indicated to enable the proportions of molybdenum and/or manganese to be disproportionately reduced for economy, while simultaneously providing the desired morphology. However, going above the maximum value of about 0.004 Wt.% is believed detrimental to toughness.

Some undesirable residual elements, such as_{'} sulfur (S) and phosphorus (P) are usually present in commercial steels. On the other hand, other residual elements, such as copper (Cu), chromium (Cr), titanium (Ti), etc. may also be present in relatively small amounts with some degree of benefit. However, all of these residual elements should be individually limited to less than 0.20 Wt.%.

A typical TTT diagram for an alloy as claimed is as illustrated in Figure 1, including a transformation start curve 10 and a transformation complete curve 12. A heat treatment processing route 14, therefor, is also shown, and it is to be noted that the processing route desirably avoids intersection with a nose portion 16 of the transformation start curve.

More particularly, the processing route 14 for making an article of the composition claimed included the initial formation of a 76 mmx76 mm (3"x3") ingot and subsequently rolling and/or forging the ingot down to a 38 mmx38 mm (1-1/2"x1-1/2") bar. The bar was heated to a preselected first temperature 18 within the austenite transformation temperature range. Preferably the bar is heated in a salt bath, desirably a nontoxic, -electrically heated chloride salt bath to the approximate preselected first temperature point 18 noted in Figure 1. The bar is maintained at such temperature for about 5 to 10 minutes to assure a substantially complete austenite microstructure.

The second step after heating the bar to the preselected first temperature 18 is to relatively rapidly cool or quench the heated bar as indicated in Figure 1 while missing the nose portion 16 of the transformation start curve 10 particular to the alloy steel composition of the present invention. If the heated bar is quenched toward a preselected second temperature 26 too slowly, a significant portion of the microstructure would be undesirably transformed to pearlite because the processing route would pass through a pearlite region 20 between curves 10 and 12 as indicated in Figure 1. If it is quenched at a slightly faster rate in a bath of a higher temperature, then an undsirable upper bainite microstructure could be formed because the processing route would pass through an upper bainite region 22 as shown in Figure 1. Thus, it may be appreciated that it is imperative to transform the austenite microstructure of the bar or similar article directly to a lower bainite microstructure by choosing a preselected cooling rate 28 sufficient for avoiding crossing of the transformation start curve 10 until reaching a preselected lower range of temperatures. Preferably, the lower end of such lower bainite range is defined by a preselected second temperature 26 located within a band of temperatures adjacent the Mₛ line 24 for the composition of elements selected in order to maximum the final hardness of the article. For example, I prefer that the preselected second temperature 26 be limited to less than about 15°C (30°F) above or below the Mₛ .line. The preselected second temperature should be above the Mₛ line if it is desired to substantially avoid transformation to martensite. However, even if such temperature is below the Mₛ line by the amount indicated, I believe that the percentage of martensite formation will be limited to less than about 10 Vol.%. The M temperature is typically about 270°C (520OF and the preselected second temperature 26 chosen was 260°C (500°F). The upper end of the lower bainite range is defined by a preselected third temperature 30 of about 350°C (660°F). If the preselected third temperature is raised to a higher temperature, the alloy may be transformed at least in part into an upper bainite microstructure with its undesirable coarser grain structure. In view of the above- stated considerations, the bar is preferably quenched in a second salt bath having the preselected second temperature 26. Preferably the bar is quenched in a nontoxic, electrically heated nitrate-nitrite salt bath at the preselected cooling rate 28 indicated in Figure 1. It is of note to appreciate that the time scale along the bottom of Figure 1 is of advantageous logarithmic form, so that in this way the cooling rate 28 approximates a substantially straight line throughout a significant portion of the first 10 seconds or so of the processing route 14. In the instant example the second salt bath was maintained at a quenchant temperature of about 260°C (500°F), and approximately 0.6 Wt.% water is added to the salt bath for greater quench severity.

The third step of the processing route 14 is to hold or maintain the bar at a relatively stable temperature between the above-mentioned lower and upper temperature reference lines 26 and 30 for a preselected period of time just prior to the transformation start curve 10 and thereafter to the transformation complete curve 12 to complete the transformation of the alloy steel to a substantially complete low temperature bainite microstructure. By this term it is meant that there is less than 10 Vol.% of retained austenite, substantially no pearlite, and less than about 10 Vol.% transformation to martensite in the subject lower bainite alloy steel. Since the hardness of the article increases as the holding temperature approaches the Mₛ line 24, it is desirable to maintain the bar or article at or adjacent the preselected second temperature 26. Such isothermal heat treat transformation is complete with the processing route 14 reaches the transformation complete curve 12. Thus, the transformation start and complete curves 10 and 12 define the left and right time-indicating boundaries of a lower bainite transformation region 32, while the lines 26 and 30 define the lower and upper temperature boundaries of the same region which varies in a range of about 250°C (482°F) to 350°C (660°F) for the subject alloy. Advantageously, the time scale along the bottom of the lower bainite transformation region 12 indicates that the length of holding time required for the first example alloy steel is only about 1800 seconds. This is a great improvement over the extended holding time period of prior art. On the other hand, for reduced hardness applications the holding time can be reduced to about 800 seconds by raising the temperatures of the second salt bath and the subsequent holding temperature to a piont adjacent the line 30 in order to save energy and time.

The fourth step of the processing route 14 not shown in the drawing, is to remove the article from the second salt bath and allow air cooling thereof at substantially ambient temperatures. Such step is taken after the transformation complete curve 12 has been breached by the processing route.

### Industrial applicability

In view of the foregoing, it can be appreciated that the through-hardened, low temperature bainitic alloy steel of the present invention exhibits physical properties that could be extremely useful for a wide number of applications including gears, bushings, bearings and the like. Particularly, it exhibits the potential for use in a power train gear having a plurality of teeth thereon for increasing gear static strength to a level of magnitude of 50%, reducing gear distortion by a level of magnitude of 75%, and maintaining equivalent pitting resistance when compared to conventional carburized and hardened steel gears at a minimal increase in cost. The subject lower bainite alloy steel is economical to produce, yet is adaptable to manufacturing procedures requiring no natural gas, for example. Moreover, the entire thermal transformation time is less than about two hours. This has been made possible to a con- siderbale extent by preselected combinations of alloying elements which have resulted in shifting the transformation start curve 10 to the right sufficient for allowing practically attainable rates of cooling for the solution, in so positioning the completion curve 12 as to reduce holding time, and in lowering the Mₛ line 24 to achieve the desired high level of hardness. For example, by the addition of carbon alone the Mₛ line is lowered about 35°C (60°F) per 0.01 Wt.% carbon to desirably allow the transformation to be achieved at relatively lower temperatures. Furthermore, the preselected amount of boron indicated is believed to increase the time available to lower the temperature of the articie being quenched to the transformation temperature, and the amount of molybdenum has a significant effect in reducing the holding time required to complete isothermal transformation to lower bainite. Significantly too, all of the preselected elements, except boron, lower the Mₛ line.

Other aspects, objects and advantages of this invention can be obtained from a study of the drawings, the disclosure and the appended claims.

## Claims

1. A bainitic steel alloy article consisting of carbon in the range of 0.65 to 0.75 Wt.%, manganese in the range of 0.60 to 0.70 Wt.%, silicon in the range of 1.20 to 2.00 Wt.%, molybdenum in the range of 0.50 to 0.60 Wt.%, optionally boron in the range of 0.0003 to 0.004 Wt.%, a plurality of residual elements individually limited to less than 0.20 Wt.% and the balance iron, said article having been heat treated to achieve a predominantly homogeneous and substa^{p}tially complete low temperature bainite microstructure.

2. The bainitic steel alloy of claim 1 including less than 10 Vol.% retained austenite in the microstructure.

3. The bainitic steel alloy article of claim 1 wherein the substantially complete low temperature bainite morphology thereof includes less than 10 Vol.% transformation to martensite.

4. The bainitic steel alloy article of claim 1 wherein boron is present in the range of 0.002 to 0.0035 Wt.%.

5. The bainitic steel alloy article of claim 1 wherein said article is austempered to directly form the low temperature bainite morphology without thermo-mechanical processing or hot/warm working.

6. The bainitic steel alloy article of claim 1 wherein said article has a composition consisting essentially of about 0.70 Wt.% carbon, 0.65 Wt.% manganese, 1.50 Wt.% silicon, 0.55 Wt.% molybdenum, 0.003 Wt.% boron, and the balance substantially iron.

7. The bainitic steel alloy article of claim 1 wherein said article has substantially not pearlite or upper bainite therein.

8. The bainitic steel alloy article of claim 1 wherein said article exhibits a hardness level above about Rc 56.

9. The bainitic steel alloy article of claim 1 wherein said article is a gear having a plurality of gear teeth thereon.

10. The bainitic steel alloy article of claim ι wherein said article is a bushing.

## Patentansprüche

1. Artikel aus bainitischer Stahl-Legierung, bestehend aus:
Kohlenstoff im Bereich von 0,65 bis 0,75 Gew.- %, Mangan im Bereich von 0,60 bis 0,70 Gew.-%, Silizium im Bereich von 1,20 bis 2,00 Gew.-%, Molybdän im Bereich von 0,50 bis 0,60 Gew.-%, wahlweise Bor im Bereich von 0,0003 bis 0,004 Gew.-%, eine Vielzahl von Restelementen einzeln beschränkt auf weniger als 0,20 Gew.-%, wobei der Rest Eisen ist, wobei der Artikel wärmebehandelt ist, um eine vorherrschend homogene und im wesentlichen vollständige Niedertemperatur - Bainitmikrostruktur zu erreichen.

2. Bainitische Stahl-Legierung nach Anspruch 1 mit weniger als 10 Vol.-% zurückbehaltenem Austenit in der Mikrostruktur.

3. Bainit-Stahllegierungsartikel nach Anspruch 1, wobei die im wesentlichen vollstädige Niedertemperatur - Bainitmorphology desselben weniger als 10 Vol.-% Transformation zu Matensit aufweist.

4. Bainit-Stahlleigierungsartikel nach Anspruch 1, wobei Bor im Bereich von 0,002 bis 0,0035 Gew.-% vorhanden ist.

5. Bainit-Stahllegierungsartikel nach Anspruch 1, wobei der Artikel der Austemperung unterworfen wurde, um direkt die Niedertemperatur-Bainitmorphology zu bilden, ohne thermomechanische Verarbeitung oder Heiß/-Warm-Bearbeitung.

6. Bainit-Stahllegierungsartikel nach Anspruch 1, wobei der Artikel eine Zusammensetzung aufweist, die im wesentlichen aus folgendem besteht:
ungefähr 0,70 Gew.-% Kohlenstoff, 0,65 Gew.- % Mangan, 1,50 Gew.-% Silizium, 0,55 Gew.-% Molybdän, 0,003 Gew.-% Bor und dem Rest im wesentlichen Eisen.

7. Bainit-Stahllegierungsartikel nach Anspruch 1, wobei der Artikel im wesentlichen kein Pearlit oder oberes Bainit darin enthält.

8. Bainit-Stahllegierungsartikel nach Anspruch 1, wobei der Artikel ein Härteniveau oberhalb ungefähr Rc 56 besitzt.

9. Bainit-Stahllegierungsartikel nach Anspruch 1, wobei der Artikel ein Zahnrad ist mit einer Vielzahl von Zahnradzähnen daran.

10. Bainit-Stahllegierungsartikel nach Anspruch 1, wobei der Artikel eine Buchse ist.

## Revendications

1. Objet en alliage d'acier bainitique comprenant du carbone dans la proportion de 0,65 à 0,75% en poids, du manganèse dans la proportion de 0,60 à 0,70% en poids, du silicium dans la proportion de 1,20 à 2,00 en poids, du molybdène dans la proportion de 0,50 à 0,60% en poids, facultativement du bore dans la proportion de 0,0003 à 0,004% en poids, un certain nombre d'éléments résiduels limités individuellement à moins de 0,20% en poids, le reste étant du fer, ledit objet ayant été traité à la chaleur pour obtenir une microstructure de bainite à basse température principalement homogène et pratiquement complète.

2. Alliage d'acier bainitique selon la revendication 1, comprenant moins de 10% en volume d'austénite retenue dans la microstructure.

3. Objet en alliage d'acier bainitique selon la revendication 1, dont la morphologie bainitique à basse température pratiquement complète comprend une transformation en martensite de moins de 10% en volume.

4. Objet en alliage d'acier bainitique selon la revendication 1, dans lequel le bore est présent dans une proportion de 0,002 à 0,0035% en poids.

5. Objet en alliage d'acier bainitique selon la revendication 1, qui a été austempéré pour former directement une morphologie bainitique à basse température sans processus thermomécanique ou traitement à une température élevée ou moyenne.

6. Objet en alliage d'acier bainitique selon la revendication 1, qui a une composition comprenant essentiellement 0,70% en poids de carbone, 0,65% en poids de manganèse, 1,50% en poids de silicium, 0,55% en poids de molybdène, 0,003% en poids de bore, le reste étant pratiquement du fer.

7. Objet en alliage d'acier bainitique selon la revendication 1, qui ne contient pratiquement pas de perlite ou de bainite supérieure.

8. Objet en alliage d'acier allié bainitique selon la revendication 1, qui présente un degré de dureté supérieur à environ Rc 56.

9. Objet en alliage d'acier bainitique selon la revendication 1, qui est un engrenage ayant un certain nombre de dents.

10. Objet en alliage d'acier bainitique selon la revendication 1, qui est un coussinet.
